

2,960,470

## METHOD OF MANUFACTURING PERMANENT MAGNETS

Robert Loosjes, Cornelis Frederik Veenemans, and Gerard Hugo Weber, Eindhoven, Netherlands, assignors, by mesne assignments, to North American Philips Company, Inc., New York, N.Y., a corporation of Delaware

No Drawing. Filed Dec. 21, 1955, Ser. No. 554,605

Claims priority, application Netherlands Dec. 21, 1954

8 Claims. (Cl. 252—62.5)

Permanent magnets which substantially consist of simple crystals or mixed crystals having a constitution according to the formula  $M_xCa_{(1-x)}0.6Fe_2O_3$ , where M is one or more of the metals Ba, Sr or Pb and  $0.6 \leq x \leq 1$ , are known (see for example French patent specification No. 1,048,792 or U.S. Patent 2,672,777, and Philips Technical Review, volume 13, No. 7, January 1952, pages 194-208). It is also known (see French patent specification 1,080,514, or U.S. Patent 2,762,778) to manufacture crystal oriented or anisotropic permanent magnets which consist of such materials. As pointed out in those patents and publications, the constituent essential to the magnetic properties of the material is  $MFe_{12}O_{19}$  or  $MO.6Fe_2O_3$ , M being barium, strontium or lead, or mixed crystals of two or more of those compounds. Calcium may be substituted for one of said metals in an amount up to 0.4 as an atomic fraction of those metals. Thus, the formula of the essential constituent may be written (to include calcium) as  $M_xCa_{(1-x)}0.6Fe_2O_3$  or



x being greater than 0.6 and less than 1. Other, and non-essential constituents may and often are present. Thus, commonly, an excess of one of the oxides, preferably the bivalent metal oxide, is employed in the starting mixture and this excess may remain as unreacted or partially reacted material in the final composition, for as noted in U.S. Patent 2,762,777, these materials may be prepared by mixing the oxides in a relatively wide range of proportions representing a significant departure from the ratio appearing in the constituent essential to the magnetic properties of the material.

As described in U.S. Patent 2,762,778, this material can be made anisotropic by orienting the crystals while they are in a mobile state. Preferably this is accomplished by suspending the material, in finely-divided form, in a liquid arranged between the poles of a magnet. The material is preferably compressed during orientation and then sintered at a temperature of about 1100 to 1450° C. to form a coherent body. This method has already led to the manufacture of permanent magnets having a  $(BH)_{max}$ -value exceeding  $2 \times 10^6$  gauss-oersted. The mechanical properties also of the magnets thus produced are generally satisfactory. However, the method concerned does not give complete satisfaction when magnets of more or less complicated shape have to be manufactured. It should be borne in mind that the dies which must be used for carrying out said method must obviously also be of complicated structure and, in addition, must be relatively water tight and mechanically strong, which properties usually are hardly compatible. That is to say, the die must be able to contain the powder in suspension so that during compacting the particles are free to move. The excess liquid which is squeezed out during compacting may be ejected from the die during or after pressing. It has been found in practice that such dies

frequently break down owing to wear when comparatively large quantities of water are drawn off.

Obviously, said difficulties can be obviated by manufacturing permanent magnets of simple shape and subsequently shaping them mechanically into the required complicated form, however, this method does not completely satisfy either, since the members concerned are not very suitable to mechanical working, for they are too hard.

- 10 As an alternative, it has been proposed in the French patent specification No. 1,080,514 mentioned hereinbefore to compress the particles of the crystal powder required to be worked up into a permanent magnet as such, that is to say without the use of any liquid, the particles 15 of the powder still retaining a certain amount of freedom of movement relative to each other, in a magnetic field (hereinafter referred to as "dry moulding method") and subsequently to sinter the produced moulding to form a permanent magnet. The mechanical properties and the 20 compactness of the permanent magnets produced so far by this method, however, are unsatisfactory.

The invention solves the problem of manufacturing anisotropic permanent magnets of the kind described and having a comparatively complicated structure, by the 25 use of a method which comprises features both of the "wet" and of the "dry" moulding method. According to the invention, one proceeds as follows. Similarly to the "wet" moulding method, the permanent magnet powder is suspended in an indifferent liquid, for example water, 30 and the liquid is removed from the suspension, for example by filtering, while the suspension is arranged between the poles of a magnet. Thus, a conglomerate is obtained which has a magnetic directive effect: it is magnetically anisotropic. The conglomerate is granulated, 35 for example by means of a sieve, through which the solid substance is pressed. The granulate produced is subsequently arranged in a moulding die in which it is compressed between the poles of a magnet. The molded product obtained, the (magnetically anisotropic) grains 40 of which due to the last operation are comparatively satisfactorily parallel oriented magnetically, finally is sintered again to form the ultimately required permanent magnet. This method permits the production of permanent magnets having a  $(BH)_{max}$ -value exceeding approximately  $1.5 \times 10^6$  gauss-oersted. Preferably the granulate, prior to being worked up into a molded product in the above-mentioned manner, has a substance added to it which imparts a satisfactory coherence to it and nevertheless does not increase the friction between the grains 50 during the molding process. Suitable substances are particularly solid organic substances which are liquefied under a slight pressure (of less than 500 kg./cm.<sup>2</sup>). Camphor or chemically related substances have proved very suitable for the purpose concerned; thus, camphor is 55 liquefied at a pressure of from 75 to 100 kg./cm.<sup>2</sup>. Preferably the camphor or similar substance is added in the form of an alcoholic solution, for example a solution of 2% by weight, which is sprayed over the granulate required to be molded. Instead of camphor or a similar 60 substance use may, for example, be made of paraffin.

In order that the invention may readily be carried out, two examples will now be described in detail.

*Example 1*

- 65 Finely powdered barium carbonate,  $BaCO_3$ , and ferric oxide,  $Fe_2O_3$ , are thoroughly mixed at a ratio of 1.1:6 mol. The mixture is compressed to form blocks and these blocks are fired for approximately 15 minutes at 1280° C. After cooling, the blocks are pulverised and the obtained powder is worked up into a suspension after the addition of a small amount of water and 1% by weight of calcium carbonate,  $CaCO_3$ . From this suspension the

water is removed by filtering in a magnetic field, after which the filter cake is dried by exposure to air. The air-dried substance is subsequently pressed through a sieve having meshes of approximately 2 x 2 mms. The grains produced are compressed in a magnetic field and finally fired for approximately 5 minutes at approximately 1250° C.

The properties of the permanent magnet produced by this method were as follows:

$B_r = 3050$  gauss

$B_{H_c} = 1450$  oersted

$I_{H_c} = 1600$  oersted

$(BH)_{max} = 1.8 \times 10^6$  gauss-oersted (at  $H = 1000$  oersted)

*Example II*

Barium carbonate,  $BaCO_3$ , and ferric oxide,  $Fe_2O_3$ , are fine powdered and thoroughly mixed at a ratio of 1.1:6 mol and fired at 1280° C. for approximately 15 minutes. The permanent magnetic reaction product is worked up into a suspension after the addition of a small amount of water and 1% by weight of calcium carbonate,  $CaCO_3$ . From this suspension the water is removed by filtering in a magnetic field, after which the filter cake produced is dried by exposure to air. The air-dried substance is pressed through a sieve having meshes of approximately 1 x 1 mm. An alcoholic solution of 2% by weight of camphor is sprayed over the grains produced. The alcohol is evaporated by exposing the granulate to air for some time. The grains mixed with camphor are subsequently compressed in a magnetic field and the molded product thus obtained is finally fired for approximately 5 minutes at approximately 1240° C.

The properties of a permanent magnet produced in this manner were as follows:

$B_r = 3340$  gauss

$B_{H_c} = 1240$  oersted

$I_{H_c} = 1280$  oersted

$(BH)_{max} = 2.3 \times 10^6$  gauss-oersted (at  $H = 1100$  oersted)

What is claimed is:

1. In the manufacture of a permanent anisotropic magnet, the steps of suspending in a chemically inert liquid crystals of a material having a composition



in which M is at least one of the metals selected from the group consisting of barium, strontium and lead, and x is at least equal to 0.6 and not greater than 1, filtering the liquid under the action of a magnetic field to thereby produce a magnetically anisotropic conglomerate, granulating the conglomerate, molding the conglomerate under the action of a magnetic field to produce a magnetically anisotropic body, and sintering said body at a temperature of about 1100° to 1400° C. to produce a highly-coherent permanent magnet body having a  $(BH)_{max}$   $1.5 \times 10^6$  gauss-oersted.

2. In the manufacture of a permanent anisotropic magnet, the steps of suspending in a chemically inert liquid crystals of a material having a composition



in which M is at least one of the metals selected from the group consisting of barium, strontium and lead, and x is at least equal to 0.6 and not greater than 1, filtering the liquid under the action of a magnetic field to thereby produce a magnetically anisotropic conglomerate, granulating the conglomerate, adding to the granulated conglomerate an organic binder adapted to increase cohesion between grains without increasing friction therebetween during molding, molding the conglomerate under the action of a magnetic field to produce a magnetically anisotropic body, and sintering said body at a temperature of about 1100° to 1400° C. to produce a highly-coherent permanent magnet body having a  $(BH)_{max}$  value exceeding approximately  $1.5 \times 10^6$  gauss-oersted.

3. In the manufacture of a permanent anisotropic magnet, the steps of suspending in a chemically inert liquid crystals of a material having a composition



in which M is at least one of the metals selected from the group consisting of barium, strontium and lead, and x is at least equal to 0.6 and not greater than 1, filtering the liquid under the action of a magnetic field to thereby produce a magnetically anisotropic conglomerate, granulating the conglomerate, adding to the granulated conglomerate an organic binder adapted to be liquefied at a pressure of less than about 500 kg./cm.<sup>2</sup> and further adapted to increase cohesion between grains without increasing friction

therebetween during molding, molding the conglomerate under the action of a magnetic field to produce a magnetically anisotropic body, and sintering said body at a temperature of about 1100° to 1400° C. to produce a highly-coherent permanent magnet body having a  $(BH)_{max}$  value exceeding approximately  $1.5 \times 10^6$  gauss-oersted.

4. In the manufacture of a permanent anisotropic magnet, the steps of suspending in a chemically inert liquid crystals of a material having a composition



in which M is at least one of the metals selected from the group consisting of barium, strontium and lead, and x is at least equal to 0.6 and not greater than 1, filtering the liquid under the action of a magnetic field to thereby produce a magnetically anisotropic conglomerate, granulating the conglomerate, adding camphor to the granulated conglomerate, molding the conglomerate under the action of a magnetic field to produce a magnetically anisotropic body, and sintering said body at a temperature of about

1100° to 1400° C. to produce a highly-coherent permanent magnet body having a  $(BH)_{max}$  value exceeding approximately  $1.5 \times 10^6$  gauss-oersted.

5. In the manufacture of a permanent anisotropic magnet, the steps of suspending in a chemically inert liquid crystals of a material having a composition



in which M is at least one of the metals selected from the group consisting of barium, strontium and lead, and x is at least equal to 0.6 and not greater than 1, filtering the liquid under the action of a magnetic field to thereby produce a magnetically anisotropic conglomerate, granulating the conglomerate, adding an alcoholic solution of camphor

to the granulated conglomerate, molding the conglomerate under the action of a magnetic field to produce a magnetically anisotropic body, and sintering said body at a temperature of about 1100° to 1400° C. to produce a highly-coherent permanent magnet body having a  $(BH)_{max}$  value exceeding approximately  $1.5 \times 10^6$  gauss-oersted.

6. In the manufacture of a permanent anisotropic magnet, the steps of suspending in a chemically inert liquid crystals of a material having a composition



in which M is at least one of the metals selected from the group consisting of barium, strontium and lead, and x is at least equal to 0.6 and not greater than 1, filtering the liquid under the action of a magnetic field to thereby produce a magnetically anisotropic conglomerate, granulating the conglomerate, spraying the granulated conglomerate with an alcoholic camphor solution, molding the conglomerate under the action of magnetic field to

produce a magnetically anisotropic body, and sintering said body at a temperature of about 1100° to 1400° C. to produce a highly-coherent permanent magnet body having a  $(BH)_{max}$  value exceeding approximately  $1.5 \times 10^6$  gauss-oersted.

7. In the manufacture of a permanent anisotropic mag-

net, the steps of suspending in a chemically inert liquid crystals of a material having a composition



in which  $M$  is at least one of the metals selected from the group consisting of barium, strontium and lead, and  $x$  is at least equal to 0.6 and not greater than 1, filtering the liquid under the action of a magnetic field to thereby produce a magnetically anisotropic conglomerate, granulating the conglomerate, adding paraffin to the granulated conglomerate, molding the conglomerate under the action of a magnetic field to produce a magnetically anisotropic body, and sintering said body at a temperature of about 1100° to 1400° C. to produce a highly-coherent permanent magnet body having a  $(BH)_{max}$  value exceeding approximately  $1.5 \times 10^6$  gauss-oersted.

8. In the manufacture of a permanent anisotropic magnet, the steps of suspending in a chemically inert liquid crystals of a material having a composition



in which  $x$  is at least equal to 0.6 and not greater than 1, filtering the liquid under the action of a magnetic field to thereby produce a magnetically anisotropic conglomerate, granulating the conglomerate, spraying the granulated conglomerate with an alcoholic camphor solution, molding the conglomerate under the action of a magnetic field to produce a magnetically anisotropic body, and sintering

said body at a temperature of about 1100° to 1400° C. to produce a highly-coherent permanent magnet body having a  $(BH)_{max}$  value exceeding approximately  $1.5 \times 10^6$  gauss-oersted.

#### References Cited in the file of this patent

#### UNITED STATES PATENTS

|    |           |                   |                |
|----|-----------|-------------------|----------------|
| 10 | 2,535,025 | Albers-Schoenberg | Dec. 26, 1950  |
|    | 2,565,861 | Leverenz          | Aug. 28, 1951  |
|    | 2,705,701 | Crowley           | Apr. 5, 1955   |
|    | 2,714,580 | Dean et al.       | Aug. 2, 1955   |
|    | 2,723,238 | Simpkiss          | Nov. 8, 1955   |
|    | 2,762,777 | Went et al.       | Sept. 11, 1956 |
|    | 2,849,312 | Peterman          | Aug. 26, 1958  |
|    | 2,854,412 | Brockman          | Sept. 30, 1958 |

#### FOREIGN PATENTS

|    |           |         |               |
|----|-----------|---------|---------------|
| 20 | 516,598   | Belgium | June 29, 1953 |
|    | 521,244   | Belgium | Jan. 6, 1954  |
|    | 1,080,514 | France  | June 2, 1954  |

#### OTHER REFERENCES

- "Elec. Eng.," July 1952, pages 644-647.  
 "Reviews of Modern Physics," vol. 25, No. 1, January 1953.  
 "Phillips Tech. Review," vol. 16, November 1954, pages 141-146.

UNITED STATES PATENT OFFICE  
CERTIFICATION OF CORRECTION

November 15, 1960

Patent No. 2,960,470

Robert Loosjes et al.

It is hereby certified that error appears in the above numbered patent requiring correction and that the said Letters Patent should read as corrected below.

Column 1, line 21, for "U. S. Patent 2,672,777" read  
-- U. S. Patent 2,762,777 --.

Signed and sealed this 9th day of May 1961.

(SEAL)

Attest:

ERNEST W. SWIDER

Attesting Officer

DAVID L. LADD  
Commissioner of Patents